

products is attempted, heavy undesirable sludges are formed. This invention permits the simultaneous application of such immiscible or incompletely miscible bituminous materials with the resultant formation of a substantially homogeneous coating or binder, since the coal tar and asphalt may be dispersed in one and the same aqueous medium even though they are incompletely miscible.

10 It will, of course, be understood that the saponifying agent, aqua ammonia, employed for saponifying the oleic acid in the example cited may be added in two successive stages; that is, part to the water used in producing the initial 15 emulsion and part to the initial emulsion itself, instead of adding all of the aqua ammonia to the water, if so desired, and a preferred soap may be used instead of soap-forming materials if preferred.

20 The term "coal tar", as used in the specification and claims, includes raw coal tar, dehydrated coal tar, and stripped coal tar from which a portion of the volatile constituents have been removed.

While I have described my invention herein 25 with particular reference to the emulsification of heavy coal tars and have referred specifically to asphalt flux oil as a bitumen suitable for use in producing the primary emulsion to which the coal tar is added, it will be understood that my invention is not limited to the use of these specific materials or to the preferred forms of my invention recited herein by way of illustration, but may be varied considerably without departing from the spirit and scope thereof.

35 I claim:

1. The method of producing a stable emulsion of coal tar and asphalt flux oil, the disperse phase of which emulsion contains a predominant amount of coal tar, which comprises adding 15 40 parts by weight of oleic acid to 250 parts by weight of asphalt flux oil, heating the mix to about 100° C., adding the same to 750 parts of water to which have been added 34 parts of aqueous ammonia whereby an emulsion of the asphalt flux oil which 45 has a viscosity substantially greater than that of water is produced, thereafter adding 1500 parts by weight of coal tar which has a specific gravity of about 1.18 or more heated to a temperature of about 70° C. to which has been added 45 parts 50 of oleic acid, vigorously agitating said tar with the emulsion of asphalt flux oil, and subjecting the resulting mixed emulsion to intensive mechanical disintegration, as for example by passage through a colloid mill.

55 2. A stable asphalt-coal tar emulsion comprising from 10 to 34 per cent asphalt, 36 to 60 per cent coal tar, 28 to 43 per cent water, and a small amount of a salt of a higher fatty acid as the emulsifying agent.

3. A method of producing a stable emulsion of coal tar and petroleum asphalt, the disperse phase of which emulsion contains a predominant amount of coal tar, which comprises mixing from 1.25 to 2.5 parts by weight of oleic acid with about 5 8 parts by weight of petroleum asphalt having a melting point of from 105 to 120° F. (ring and ball method), adding this mixture while stirring to about 30 parts by weight of hot water containing ammonia in an amount more than sufficient to neutralize the oleic acid, thus forming an emulsion of asphalt in water, and gradually adding to this emulsion about 60 parts by weight of liquefied coal tar having a melting point of approximately 80° F. 10 15

4. A bitumen emulsion comprising from 10 to 34 per cent of easily emulsifiable asphaltic bituminous material, from 36 to 60 per cent of coal tar having a specific gravity of about 1.15 or higher at 25° C., from 28 to 43 per cent of water, and 20 a small amount of a salt of a higher fatty acid as the emulsifying agent.

5. The method of producing a substantially stable dispersion containing as the disperse phase 25 a relatively large amount of tar of the group consisting of coal tar and water gas tar of a specific gravity of at least 1.15 and a smaller amount of asphalt, which comprises producing an initial dispersion containing an aqueous medium, soap and a relatively small amount of asphalt and thereafter dispersing tar of the group consisting of 30 coal tar and water gas tar in amount greater than the amount of asphalt directly in said initial dispersion.

6. A substantially stable dispersion of asphaltic 35 bitumen and tar of the group consisting of coal tar and water gas tar in an aqueous medium, the disperse phase of said dispersion containing a minor proportion of asphaltic bitumen and a major proportion of tar of the group consisting of 40 coal tar and water gas tar, said dispersion containing at least about 28 percent of water and an emulsifying agent.

7. The process of producing a stable dispersion, 45 the disperse phase of which is constituted predominantly of tar of the group consisting of coal tar and water gas tar, in an aqueous medium, comprising producing an initial emulsion containing a relatively small amount of asphaltic bitumen in an aqueous dispersing medium, and an emulsifying agent, and adding an amount of tar of the group consisting of coal tar and water gas tar greater than the amount of said asphaltic bitumen to said initial emulsion to form the said 50 stable dispersion, the disperse phase of which is predominantly constituted of said tar. 55

WILLIAM FRANCIS FAIR, JR.



## UNITED STATES PATENT OFFICE

2,087,401

PROCESS OF MAKING BITUMINOUS  
EMULSIONS

William F. Fair, Jr., New York, N. Y., assignor to  
The Barrett Company, New York, N. Y., a cor-  
poration of New Jersey

No Drawing. Application February 9, 1934,  
Serial No. 710,533

2 Claims. (Cl. 134—1)

This invention relates to emulsions or dis-  
persions of bituminous materials, and more par-  
ticularly, to coal tar emulsions and methods for  
producing the same.

Heretofore, emulsions of asphalts have been  
made and used for surfacing roads, curing con-  
crete, protecting iron work, etc. In some in-  
stances, light tars have also been emulsified.  
Heavy coal tars, that is coal tars having a specific  
10 gravity of from 1.18, or even as low as 1.15, to  
1.25 or higher at 25° C. have not been success-  
fully used in producing emulsions prior to the in-  
vention of my copending application Serial No.  
628,113, filed August 9, 1932, for the reason that  
15 emulsions of such tars when produced by proc-  
esses such as are used in producing asphaltic  
emulsions are relatively unstable so that the tar  
soon settles out of suspension.

Coal tars generally are of higher specific  
20 gravity than asphalts and this property may ac-  
count, in part at least, for the comparative in-  
stability of emulsions or dispersions of coal tars  
as heretofore produced. Among the factors  
25 which influence the stability of emulsions and  
tend to cause settling out of the material dis-  
persed are differences in density of the disperse  
phase and the continuous phase and differences  
in viscosity of the two phases or a combination  
30 of these factors with others. It has been pro-  
posed to increase the stability of emulsions or  
dispersions of bituminous materials by (1) in-  
creasing the density of the aqueous phase and (2)  
by decreasing the density of the disperse phase.  
Method (1) has been practiced heretofore by  
35 adding clay or the like to the aqueous phase prior  
to the dispersion of the bituminous material.  
However, the resulting dispersion then contains  
undesired inert inorganic material. Method (2)  
has been used by cutting back the bituminous  
40 material with a sufficient amount of a light  
organic solvent to reduce the density and viscosity  
of the material dispersed. This method, it will  
be noted, requires the use of substantial amounts  
of relatively expensive solvents and changes the  
45 physical properties of the bituminous phase.

Among the objects of this invention are to  
produce bituminous emulsions of improved sta-  
bility, and particularly, coal tar emulsions or dis-  
persions of improved stability; to provide an in-  
50 expensive and simple method by which such emul-  
sions or dispersions can be made and to produce  
such emulsions without incorporating objection-  
able inert inorganic materials therein. These  
and other objects of this invention will appear  
55 from the following description thereof.

In my copending application, hereinabove re-  
ferred to, there is disclosed a procedure of mak-  
ing coal tar emulsions involving the formation  
of an initial emulsion by dispersing a relatively  
small amount of a suitable easily-emulsifiable  
5 bituminous material, such as asphalt, in an  
aqueous medium and then adding to this initial  
emulsion relatively heavy coal tar or water gas  
tar. Asphalts, asphalt flux oil, petroleum, fuel  
oil, or other asphaltic or petroleum bitumens may  
10 be employed as the bituminous material for the  
disperse phase of the initial emulsion. Prefer-  
ably, asphalt having a penetration at 77° F. of  
from 100 to 220 tenths of a millimeter (deter-  
mined by A. S. T. M. Standard Method D5-25) is  
15 utilized. A relatively heavy coal tar having a  
specific gravity of not less than 1.15 at 25° C.  
and a viscosity of not less than approximately  
60 seconds for 100 c. c. at 100° C. or a relatively  
heavy water gas tar having a viscosity of not less  
20 than approximately 60 seconds per 100 c. c. at  
100° C. is dispersed in the initial emulsion.  
Heavier and more viscous coal tars, including  
coke oven, vertical and horizontal retort tars,  
water gas tar, or other relatively heavy bituminous  
25 material of different characteristics from that  
forming the disperse phase of the initial emul-  
sion may be added to the initial emulsion.

In producing such emulsions, preferably a soap  
or saponaceous material is employed as a dis-  
persing agent to aid in the production of both  
30 the initial and the final emulsion. The soap-  
forming materials may be added to the aqueous  
medium and to the bituminous material to be  
dispersed so that a reaction between the soap-  
35 forming materials which results in the forma-  
tion of soap takes place during the emulsification  
of the bituminous material. Preferably, the  
basic constituent of the soap is added to the  
aqueous medium in which it is readily soluble and  
40 the acidic constituent is added to the material  
to be dispersed, although, if desired, the soap  
emulsifier, as such, or soap-forming constituents  
may be added to the emulsion during its forma-  
45 tion or immediately after the addition of the  
bituminous material to the aqueous medium and  
during the agitation of the mixture. Ammonium  
or sodium soaps of fatty acids or mixtures of  
fatty acids, sodium resinate, the reaction prod-  
50 uct of sodium silicate and oleic acid, the sodium  
salts of sulfonated coumarone resin and associated  
sulfonated coumarone-like compounds or the  
sodium salts of other sulfonated benzene deriva-  
tives may be employed as dispersing agents.

Emulsions of asphalts and readily emulsifiable